

Dec. 20, 1960

H. B. BOMBERGER ET AL

2,965,521

METAL PICKLING SOLUTIONS AND METHODS

Original Filed June 10, 1954

EFFECT ON HYDROGEN ABSORPTION OF VARYING  
NITRIC ACID CONTENT IN REMOVING 0.004 INCH  
OF METAL FROM A Ti-7% Mn. ALLOY IN AN AQUEOUS  
PICKLING BATH CONTAINING 2% OF HYDROFLUORIC  
ACID, AT A BATH TEMPERATURE OF 150°F.



INVENTORS.  
HOWARD B. BOMBERGER,  
BY MILTON B. VORDAHL.

Ward Heath Haseltine Omer McElhanon  
ATTORNEYS.

1

2,965,521

## METAL PICKLING SOLUTIONS AND METHODS

Howard B. Bomberger, East Liverpool, Ohio, and Milton B. Vordahl, Beaver, Pa., assignors, by mesne assignments, to Crucible Steel Company of America, Flemington, N.J., a corporation of New Jersey

Original application June 10, 1954, Ser. No. 435,755. Divided and this application Nov. 16, 1956, Ser. No. 622,662

4 Claims. (Cl. 134—3)

This invention pertains to improvements in pickling solutions and in methods of pickling metals to remove surface scale, oxides or other surface contaminations.

The present application is a division of our copending application for United States Letters Patent Serial No. 435,755, filed June 10, 1954.

The invention is particularly applicable to the pickling of metals like titanium, zirconium and their alloys, which are subject to serious surface embrittlement, due to absorption of oxygen, nitrogen, hydrogen, etc., when heated in air to elevated temperatures, such as those required for heat treating or for hot rolling or forging operations or the like. Removal of this embrittled surface layer, as by acid pickling, improves ductility, particularly bend ductility.

Most acids do not, however, readily attack corrosion resistant metals like titanium, zirconium and the majority of their alloys in which titanium or zirconium is the major constituent. And among those which do, the majority hydrogen-embrittled and/or deeply pit the surfaces of the metal.

In accordance with the present invention, we have discovered that notable exceptions to the above, are appropriate concentrations of hydrofluoric acid or equivalent amounts of fluoride salts when employed in aqueous pickling solutions containing strong oxidants, such as nitric acid or hydrogen peroxide or both in critically controlled amounts.

The present method of pickling titanium and titanium alloys is to use the conventional steel plant pickling bath comprising an aqueous solution containing about 10% by weight of nitric acid and 2% of hydrofluoric acid and maintained at about 160° F. for removing from about 0.002" to 0.004" of metal from the surface in about 2 to 20 minutes.

The major disadvantages of this practice are: (1) Substantial amounts of hydrogen are absorbed by the metal resulting in serious loss of ductility; (2) copious quantities of the hazardous nitrogen dioxide gas are evolved which sometimes exceeds available ventilating capacity; and (3) the bath is difficult to control. Rapid depletion results in dangerously low concentrations of nitric acid.

The dissolution of metals in aqueous pickling solutions is basically an electrochemical phenomenon resulting in the formation of metallic ions. This is known as an oxidation reaction, e.g., in the case of titanium in a reducing acid,



A necessary requirement for this reaction to proceed is the simultaneous reduction of either cations or an oxidizing agent—a reduction reaction. In a reducing solution, hydrogen ions are reduced, resulting in the formation of atomic and molecular hydrogen, i.e.,



2

and



Thus, if a metal is picked in a reducing acid solution such as hydrogen fluoride, hydrogen ions are reduced and atomic hydrogen diffuses into the metal. With metals such as titanium, this results in a serious loss in ductility. Thus



However, if a cation or an oxidizing agent is present which is more readily reduced than hydrogen ions, no hydrogen is evolved or absorbed by the metal. For example, on pickling titanium in an acid solution containing fluoride ions and hydrogen peroxide, the peroxide is reduced to water along with the formation of a titanium fluoride complex.



And, on pickling titanium in a nitric acid solution containing fluoride ions, the nitric acid is reduced, forming a titanium fluoride complex, water and colorless nitric oxide (NO). The probable reaction is:



The nitric oxide is immediately oxidized to the brown, poisonous nitrogen dioxide on exposure to air, i.e.,



The dioxide is very soluble in water, forming nitric acid and nitric oxide, which can also be oxidized to the dioxide, thus forming nitric acid, e.g.,



If the concentration of the oxidant is too low, the reduction of hydrogen ions may occur along with the reduction of the oxidizing agent. The rate of a given such reaction is a function of concentration and mobility of reactants and products, changes of free energy and other factors. In this case there is some absorption and evolution of hydrogen. This condition is illustrated in the graph of the accompanying drawing in which the percent hydrogen absorbed on pickling 0.004" from Ti-7Mn sheet at 150° F. is plotted as ordinates against the nitric acid content as abscissae for an aqueous pickling solution containing 2% hydrofluoric acid in addition to nitric acid. It will be noted therefrom, that below concentrations of 15% HNO<sub>3</sub>, substantial amounts of hydrogen are absorbed.

In accordance with the present invention, the most desirable pickles are found to consist of aqueous solutions of strong water-soluble oxidants and hydrofluoric acid in concentrations of about 1/2 to 10% of the fluoride ion, i.e., about 1/2 to 10% of hydrofluoric acid or equivalent amounts of fluoride salts, such as NaF, NaBF<sub>4</sub>, etc. These pickling solutions are best used at temperatures between 100° and 190° F. Other specific conditions follow:

Aqueous solutions containing from 15 to 50% HNO<sub>3</sub> and 0.5 to 10% of fluoride ions, give a good finished surface and, as indicated in the attached figure, a minimum absorption of hydrogen. An aqueous pickling solution containing about 30% nitric acid and 4% hydrofluoric acid has been found to give exceedingly good results. It dissolves about 0.001" in a minute at 150° F. and results in very little hydrogen evolution and absorption by the metal. Below a concentration of 0.005% H, damage to the metal is so slight as to be negligible. Thus, from the accompanying graph it is clear that 15% is the minimum HNO<sub>3</sub> content for safe operation. No reduction in hydrogen pickup is noted above 30% HNO<sub>3</sub>. Increases of HNO<sub>3</sub> beyond 50% are uneconomical. The

most objectionable feature to  $\text{HNO}_3$  type pickling solution is the evolution of the poisonous  $\text{NO}_2$  gas. This is especially hazardous wherever the ventilating facilities are not adequate. The major advantage is the prevention of hydrogen absorption and thus brittleness.

Pickling solutions containing from 0.5 to 5% fluoride ions and from 5 to 35% hydrogen peroxide ( $\text{H}_2\text{O}_2$ ) also impart good surface finish to the metal and result in little hydrogen pickup. The major advantage of this type of pickling solution is that no poisonous or otherwise objectionable gases are given off by the bath. The products of reaction are simply water and a titanium complex. Optimum results are obtained with an aqueous bath containing about 20%  $\text{H}_2\text{O}_2$  and 2% fluoride ions. At 150° F. this bath pickles off about 0.001" of metal per minute. Lower temperatures are often preferred to minimize decomposition of the  $\text{H}_2\text{O}_2$ .

Aqueous solutions containing from 2 to 50%  $\text{HNO}_3$ , 0.5 to 30%  $\text{H}_2\text{O}_2$  and 0.5 to 10% fluoride ions are especially attractive. Solutions of this type give excellent surfaces and very little hydrogen pickup, and are also the most economical and do not fume. Optimum results are obtained with such solutions containing about 20%  $\text{HNO}_3$ , 2%  $\text{H}_2\text{O}_2$  and 2% fluoride ions. This concentration of  $\text{HNO}_3$  assures very little hydrogen pickup, and the  $\text{H}_2\text{O}_2$  prevents fuming by oxidizing the NO to  $\text{NO}_2$  and thus to  $\text{HNO}_3$  before it leaves the pickling solution—as little as 0.5%  $\text{H}_2\text{O}_2$  is effective.

The advantages to be derived from hydrogen peroxide additions are: (1) the prevention of NO and thus  $\text{NO}_2$  evolution to the air ( $\text{NO}_2$  is not only obnoxious but poisonous; 0.01% has been fatal); (2) it results in little or no loss of nitric acid; (3) it therefore eliminates the problem of nitric acid control; and (4) it eliminates staining of the metal sheet by  $\text{NO}_2$  on withdrawing the sheet from the bath. The presence of a surplus of  $\text{H}_2\text{O}_2$  is indicated by the color, since  $\text{H}_2\text{O}_2$  added to a solution containing titanium salts imparts a color varying from yellow to deep red with increasing  $\text{H}_2\text{O}_2$  content. This greatly simplifies control. Modifications of the three types of pickling solutions mentioned embrace the use of other oxidants, including the aeration of the solution with air, oxygen or ozone, in order to minimize the escaping of NO and  $\text{NO}_2$ .

The previously mentioned solutions can be modified to advantage by the addition of about 0.1% of a suitable wetting agent (e.g., Queen #5 by Quaker State, or Actival 57 by Haas Miller Corp.) A specific advantage is the prevention of vertical striations, which results from nonuniform pickling due to the rapid vertical movement of gas bubbles and solution along the sheet surface. The

use of a wetting agent increases the fuming from  $\text{HNO}_3\text{-HF}$  pickles but this is no problem if  $\text{H}_2\text{O}_2$  is employed in the solution or if the ventilation is adequate.

What is claimed is:

- 5 1. An aqueous solution for pickling and removing surface metal without embrittling the underlying surface of a metal selected from the group consisting of titanium, zirconium, titanium base alloys and zirconium base alloys, containing in percentages by weight about 0.5 to 10% fluoride ions, about 2 to 50% of nitric acid and about 0.5 to 30% of hydrogen peroxide.
- 10 2. The method of pickling a metal selected from the group consisting of titanium, zirconium and alloys of each with removal of metal from the surface, which comprises: immersing the metal in an aqueous pickling solution containing in percentages by weight, about 0.5 to 10% of fluoride ions and at least one member selected from the group consisting of 5 to 35% hydrogen peroxide, and 2 to 50% nitric acid together with 0.5 to 30% hydrogen peroxide, while maintaining said solution at a temperature of about 100° to 190° F.
- 15 3. The method of pickling a metal selected from the group consisting of titanium, zirconium and alloys of each with removal of metal from the surface, which comprises: immersing the metal in an aqueous pickling solution containing in percentages by weight, about 0.5 to 5% of fluoride ions, and about 5 to 35% of hydrogen peroxide, while maintaining said solution at a temperature of about 100° to 190° F.
- 20 4. The method of pickling a metal selected from the group consisting of titanium, zirconium and alloys of each with removal of metal from the surface, which comprises: immersing the metal in an aqueous pickling solution containing in percentages by weight, about 0.5 to 10% of fluoride ions, about 2 to 50% of nitric acid and about 0.5 to 30% of hydrogen peroxide while maintaining said solution at a temperature of about 100° to 190° F.
- 25 5. The method of pickling a metal selected from the group consisting of titanium, zirconium and alloys of each with removal of metal from the surface, which comprises: immersing the metal in an aqueous pickling solution containing in percentages by weight, about 0.5 to 10% of fluoride ions, about 2 to 50% of nitric acid and about 0.5 to 30% of hydrogen peroxide while maintaining said solution at a temperature of about 100° to 190° F.
- 30 6. The method of pickling a metal selected from the group consisting of titanium, zirconium and alloys of each with removal of metal from the surface, which comprises: immersing the metal in an aqueous pickling solution containing in percentages by weight, about 0.5 to 10% of fluoride ions, about 2 to 50% of nitric acid and about 0.5 to 30% of hydrogen peroxide while maintaining said solution at a temperature of about 100° to 190° F.
- 35 7. The method of pickling a metal selected from the group consisting of titanium, zirconium and alloys of each with removal of metal from the surface, which comprises: immersing the metal in an aqueous pickling solution containing in percentages by weight, about 0.5 to 10% of fluoride ions, about 2 to 50% of nitric acid and about 0.5 to 30% of hydrogen peroxide while maintaining said solution at a temperature of about 100° to 190° F.

40 References Cited in the file of this patent

UNITED STATES PATENTS

|           |                  |                |
|-----------|------------------|----------------|
| 2,542,727 | Theuerer         | Feb. 20, 1951  |
| 2,577,803 | Pfann            | Dec. 11, 1951  |
| 2,606,960 | Little           | Aug. 12, 1952  |
| 2,653,134 | Dilling et al.   | Sept. 22, 1953 |
| 2,724,667 | MacPherson       | Nov. 22, 1955  |
| 2,790,738 | Alexander et al. | Apr. 30, 1957  |

FOREIGN PATENTS

|            |               |               |
|------------|---------------|---------------|
| 50 375,599 | Great Britain | June 30, 1932 |
| 1,085,933  | France        | Oct. 19, 1955 |